

# United States Patent Office

2,734,870

Patented Feb. 14, 1956

2,734,870

## NON-SOAP SYNTHETIC DETERGENT BAR

Allen H. Lewis, Berkeley, Calif., assignor to California Research Corporation, San Francisco, Calif., a corporation of Delaware

No Drawing. Application May 21, 1951,  
Serial No. 227,507

3 Claims. (Cl. 252—161)

The invention relates to a new and useful detergent composition. More particularly, it relates to a detergent composition which can be cast, molded, or framed in conventional manner to produce a detergent bar having superior properties.

In recent years synthetic detergents, particularly the alkyl-aryl sulfonate detergents of the type described in Lewis' U. S. Patent No. 2,477,383, have won wide acceptance in household applications and very large volumes of these materials are currently manufactured and sold. These synthetic detergents have been prepared for the consumer in powdered or granular form and substantially all of these materials have been marketed in that form. The desirability of producing a synthetic detergent bar has long been recognized and extensive experimental work has been directed to this end as evidenced, for example, by McCutcheon's paper entitled "Synthetic Detergents in Bar Form," Soap, December 1949, page 33 et seq. Despite intense effort in this direction by a large number of skilled research workers, no satisfactory synthetic detergent bar has been produced which has met with wide consumer acceptance. The principal problem encountered in an effort to produce a synthetic detergent bar is that of finding a binder which would hold the active detergent components together and give the bar suitable physical characteristics. An acceptable bar should be firm, cohesive, smooth and pleasant to the touch, lather and suds well in hot and cold water, and be resistant to water in the sense that it does not become soft and slimy in use or waste away rapidly when wet, or crumble and develop abrasive areas on its surface after initial use.

It is an object of this invention to provide a synthetic detergent composition which, in bar form, meets the above indicated physical property requirements in a remarkably satisfactory manner.

It is a further object of this invention to provide a process for producing this detergent composition.

As its broadest aspect, this invention lies in the finding that a detergent composition consisting predominantly of an intimate mixture of 30 to 70 parts by weight of paraffin wax and 70 to 30 parts by weight of an organic sulfuric reaction product type detergent which is soluble in paraffin wax at a temperature in the range 200-350° F. can be cast, molded, or framed to form a synthetic detergent bar having excellent physical and deterutive properties.

These compositions are produced by melting paraffin wax and heating it to a temperature in the range 200 to 350° F., preferably 250 to 325° F., and stirring the organic sulfuric reaction product type detergent into the hot molten wax to form a clear, transparent liquid solution, and cooling the solution until it solidifies.

In a preferred embodiment of the invention, the detergent composition contains 40 to 60 parts by weight of paraffin wax and in addition to the wax and organic sulfuric reaction product type detergent a small amount

not exceeding about 10% by weight based on the total detergent composition of a polar organic compound, especially of a higher fatty acid.

In producing the preferred composition, the wax is melted and heated to a temperature in the range about 250 to 325° F. as indicated above, the higher fatty acid is added to the hot molten wax, and the organic sulfuric reaction product type detergent is then dissolved in the hot mixture.

10 Three important advantages attend the use of an organic polar compound in this manner. First, the organic sulfuric reaction product type detergent dissolves in the wax much more readily and much more rapidly with considerably less agitation to produce a solution of lowered viscosity; second, any tendency of the organic sulfuric reaction product to drop out of solution during cooling of the hot mixture and to agglomerate, forming appreciably large particles of detergent material in the bars produced and thus to render them macroscopically heterogeneous, is suppressed; and, third, the solid detergent bars produced are plasticized by the polar material.

The compositions of both of the above embodiments derive their primary valuable characteristics from the wax and organic sulfuric reaction product type detergent components. The presence of the polar material considerably simplifies the process of making the detergent compositions and enhances the already thoroughly acceptable properties of the product. The compositions of both of the above embodiments have a reasonable tolerance for the incorporation of inorganic builders which, although insoluble, may be dispersed in the bar to improve the over-all deterutive action; operable bars may contain up to about 25% by weight of any of the usual inorganic builders such as alkali metal sulfates, alkali metal phosphates, alkali metal polyphosphates and alkali metal silicates. It is preferable, however, to keep the inorganic salt content of the finished bar below about 12% of its total weight in order to avoid a tendency toward frosting, i. e., the formation of inorganic salt crystals on its surface.

45 The preferred wax for use in compounding the compositions of the invention is preferably a paraffin wax derived from petroleum having a melting point above about 125° F. and having a relatively low oil content, desirably below about 2% by weight. The wax may be either crystalline or amorphous and its melting point may range up to about 175° F. The ordinary de-oiled petroleum waxes of commerce are entirely satisfactory for compounding the detergent compositions of the invention. It should be understood that modifications of the characteristics of paraffin wax by the incorporation of small amounts of vegetable waxes is not precluded.

50 As indicated above, the active deterutive component of the composition is a water-soluble salt of an organic sulfuric reaction product which is soluble in paraffin wax at a temperature in the range about 200-350° F. These products are characterized by a large hydrophobic group consisting almost entirely of hydrocarbon material and the smaller hydrophilic sulfuric acid residue. The metal component of a salt of the organic sulfuric reaction product is ordinarily sodium, but other alkali metals and alkaline earth metals, especially magnesium, may be present as the metallic component. Materials of this general description have the common property of remaining highly dispersed 55 in the wax matrix when the composition is cold, so that the finished solid is characterized by macroscopic homogeneity.

A very considerable number of organic sulfuric reaction product type synthetic detergents are described in the literature and several of these materials are articles of commerce produced in substantial volume, for example alkyl sulfates containing 10 to 20 carbon atoms in the

## 3

alkyl group, alkyl sulfonates containing 10 to 20 carbon atoms in the alkyl group, sulfated monoglycerides of coconut oil fatty acids and especially alkyl aryl sulfonates containing 10 to 20 carbon atoms in the alkyl side chain. While these materials have similar physical properties in that they are water soluble and exhibit detergents and wetting properties and a structural similarity in that they are all characterized by a large hydrophobic group consisting almost entirely of hydrocarbon material and a smaller hydrophilic sulfuric acid residue, they are not all suitable for use as components of the compositions of this invention. To be useful here the organic sulfuric reaction product type detergent must be soluble in hot paraffin wax. Some of these materials are soluble and some are not. Without exception it has been found that those which are soluble in the wax remain highly dispersed in the wax matrix when the solution is cooled until the wax solidifies and that the solid is macroscopically homogeneous. The solubility of any particular organic sulfuric reaction product type detergent, and hence its suitability for use in composing the compositions of this invention, is readily determined by melting paraffin wax, heating it to about 300° F. and stirring the detergent into the wax. Suitable detergents dissolve in the wax forming a clear transparent liquid solution at concentrations above 30% by weight.

Organic sulfuric reaction product type detergents having a branched alkyl group containing 10 to 20 carbon atoms, especially the alkyl aryl sulfonates described in Lewis Patent 2,477,383, are highly soluble in paraffin wax. The Lewis detergent is prepared by polymerizing propylene, separating a polypropylene fraction boiling from about 325 to 520° F., alkylating a mononuclear aromatic hydrocarbon such as benzene, toluene or xylene with the polypropylene, sulfonating the alkyl aromatic hydrocarbon product and neutralizing the resultant sulfonic acid with an alkali metal hydroxide or with an alkaline earth metal hydroxide.

The organic polar material which is desirably incorporated in the preferred composition of the invention is preferably a higher fatty acid, i. e., aliphatic monocarboxylic acid containing 10 to 20 carbon atoms, for example stearic acid, oleic acid, palmitic acid and lauric acid.

As indicated above, the wax-synthetic detergent compositions of the invention will tolerate the addition of fairly substantial amounts of inorganic builders without too much sacrifice of their desirable bar-form properties. For example, the alkali metal carbonates, phosphates, borates, and silicates which are generally known as alkaline builders can be tolerated up to a maximum amount of about 25% by weight of the total bar. Neutral builders such as sodium sulfate and sodium chloride can be tolerated in similar amounts. Those skilled in the art will recognize that perfume, coloring matter and fillers such as infusorial earth and bentonite and the allied group of clays may be incorporated in the finished bar. It must be recognized that the incorporation of insoluble material will proportionately increase the viscosity of the molten mix during the preparation of the product. The term "consisting essentially" employed in the appended claims is used in the sense that conventional fillers, builders, perfumes, etc., may be added to the wax-detergent compositions.

To prepare the compositions of the following examples paraffin wax was melted and heated to a temperature in the range about 250 to 325° F., and preferably in the range 275 to 300° F., and the synthetic detergent was stirred into the wax to dissolve it. At temperatures below 200° F. the rate of solution and solubility of the detergent in the wax are low and the detergent-wax mixtures prepared at such temperatures tend to be macroscopically heterogeneous when cooled. At temperatures much above 300° F. the synthetic detergent tends to char, and color of the ultimate product is poor. The temperature preferably should not exceed 325° F. When only wax and the synthetic detergent were employed in making the

## 4

detergent composition, extensive agitation and the application of shearing force to the mixture was required to achieve homogeneity of the product. The addition of a higher fatty acid to the molten wax prior to the addition of the synthetic detergent greatly facilitated the dissolving of the detergent and brought about a marked reduction in the viscosity of the solution. After the detergent is dissolved in the wax the molten mixture may be poured into individual bar molds, or poured into a conventional frame and cooled until the mass solidifies, after which the mass is cut into bars. Alternatively, the mass may be cooled to a temperature just below its solidification point and then extruded or pressed into bars.

## Example 1

70 parts by weight of de-oiled paraffin wax having a melting point of 125° F. and an oil content below 2% by weight were heated to 310° F. 30 parts by weight of a sodium alkyl benzene sulfonate containing 12 to 15 carbon atoms in the alkyl chain were dissolved in the wax. Solution was accomplished by stirring the mixture for about 6 minutes. The fluidity of the solution was approximately that of hot molten wax. The solution was poured into a metal bar mold and cooled to room temperature. The bar separated from the mold without adhering to the metal. The bar was a light buff color and was similar to wax in consistency. The bar was smooth and pleasant to the touch, was perfectly homogeneous to visual inspection, and floated in water. When the bar was worked with the hands in the usual manner with hot or cold water, it lathered, but rather poorly.

## Example 2

60 parts by weight of the paraffin wax of Example 1 were heated to 300° F. 40 parts by weight of sodium polypropylene benzene sulfonate containing 12 to 15 carbon atoms in the polypropylene radicals were dissolved in the molten wax. The wax was cast in bar form as in Example 1. The lathering properties of this bar were considerably better than those of the bar in Example 1. The specific gravity of this bar was slightly less than 1.

## Example 3

45 47.5 parts by weight of the paraffin wax of Example 1 were melted and heated to 300° F. 52.5 parts by weight of a mixture of sodium polypropylene benzene sulfonate containing 12 to 15 carbon atoms in the polypropylene groups and sodium sulfate were incorporated in the molten wax. The ratio of sulfonate to sulfate in the solute was 60:40. The liquid dispersion produced had a considerably higher viscosity than the solutions of Examples 1 and 2 due to the salt content. The mixture was barely pourable at 300° F. The mixture was cast in bar form as in Example 1. The bar lathered well in hot and cold water, but frosted slightly after wetting because of the sodium sulfate content.

## Example 4

60 47.6 parts by weight of the wax of Example 1 were melted and heated to about 300° F. 9.6 parts by weight of palmitic acid were dissolved in the molten wax and then 42.8 parts by weight of a mixture of sodium polypropylene benzene sulfonate containing 12 to 15 carbon atoms in the polypropylene radicals and sodium sulfate were incorporated in the wax-acid solution. The ratio of sulfonate to sulfate in the latter solute was 90:10. The resulting dispersion was highly fluid and the apparent rate of solution of the sulfonate in the wax was rapid, the sulfonate apparently dissolving completely after 2 minutes of stirring. The resulting mixture was cast in bar form. The bar lathered well, but the foam broke more rapidly than the foams produced by the bars in Examples 1 to 3 inclusive, presumably because of the high fatty acid content of the bar.

## Example 5

52.4 parts by weight of the paraffin wax of Example 1 were melted and heated to about 300° F. 4.8 parts by weight of palmitic acid were dissolved in the molten wax and then 42.8 parts by weight of the sulfonate-sulfate mixture of Example 4 were incorporated in the wax-acid solution. The resultant mixture was cast in bar form. The resultant bar lathered well and the foam was more stable than the foam produced by the bar of Example 4, but not quite as stable as the foam produced by the bar of Example 2.

## Example 6

56.2 parts by weight of the paraffin wax of Example 1 were melted and heated to about 300° F. One part by weight of palmitic acid was dissolved in the molten wax and then 42.8 parts by weight of the sulfonate-sulfate mixture of Example 4 were incorporated in the wax-acid solution. The presence of the palmitic acid in this small amount noticeably increased the apparent rate of solution of the sulfonate and lowered the viscosity of the resulting mixture. The final mixture was cast in bar form. The bar lathered well in both hot and cold water and the foam produced was apparently identical with the foam produced by the bar of Example 2 with respect to stability.

## Example 7

52.3 parts by weight of the wax of Example 1 were melted and heated to about 300° F. 1.8 parts by weight of palmitic acid were dissolved in the molten wax and then 40.6 parts by weight of the sulfonate-sulfate mixture of Example 4 were incorporated in the solution. 5.3 parts by weight of glycerine were incorporated in the resultant mixture. The final mixture was cast in bar form. This bar was similar in all of its properties to the bar produced in Example 6.

## Example 8

57.7 parts by weight of a de-oiled paraffin wax having a melting point of 143° F. were melted and heated to about 300° F. 42.3 parts by weight of the sulfonate-sulfate mixture of Example 4 were incorporated in the molten wax. The mixture was cast in bar form. The bar lathered well in both hot and cold water.

## Example 9

35 parts by weight of the paraffin wax of Example 1 were melted and heated to about 300° F. 5 parts by weight of palmitic acid were dissolved in the molten wax and then 60 parts by weight of the sulfonate-sulfate mixture of Example 4 were incorporated in the solution. The final mixture was cast in bar form. This bar had excellent lathering properties, and was apparently equal in this respect to a good grade of toilet soap. During prolonged use, the bar wore away smoothly and showed no tendency to soften or crumble when exposed to the usual conditions of household use.

## Example 10

45 parts by weight of the paraffin wax of Example 1 were melted and heated to about 300° F. 5 parts by weight of stearic acid were dissolved in the molten wax

and then 50 parts by weight of an alkyl aryl sulfonate prepared by alkylating benzene with a propylene polymer fraction boiling over the range about 360 to 520° F., sulfo-nating the alkylate, and neutralizing the resultant sulfonic acid with sodium hydroxide, were dissolved in the wax-acid mixture. The resultant solution was cast in bar form. This bar had excellent lathering properties and was durable in ordinary household use.

The bars prepared in all of the foregoing examples were macroscopically homogeneous as they left the mold and all of them retained their homogeneous appearance throughout prolonged use, with the exception of the bar produced in Example 3 which showed a tendency to frost. The materials of which each of the exemplified bars are formed do not appear to wet the surfaces of metallic molds and are readily freed from the mold when cooled. The exemplified bars may be remelted and recast without loss of homogeneity and apparently without change in any of the physical or chemical properties of the composition.

I claim:

1. A firm, cohesive and macroscopically homogeneous detergent bar consisting essentially of 40 to 60 parts by weight of paraffin wax, 2 to 5 parts by weight of a fatty acid containing 10 to 20 carbon atoms per molecule and 60 to 40 parts by weight of a mixture of water-soluble alkyl aryl sulfonates, the alkyl groups being propylene polymers containing predominantly from 12 to 15 carbon atoms.

2. A firm, cohesive, macroscopically homogeneous detergent bar consisting essentially of 40 to 60 parts by weight of paraffin wax, 60 to 40 parts by weight of an alkyl benzene sulfonate detergent having 10 to 20 carbon atoms in its alkyl group, 1 to 10 parts by weight of a fatty acid containing 10 to 20 carbon atoms per molecule, and from 1 to 25 parts by weight of a water-soluble inorganic builder.

3. A process for producing a macroscopically homogeneous detergent bar which comprises forming a mixture of molten paraffin wax and a higher fatty acid, heating the mixture to a temperature in the range 250 to 325° F., dissolving an alkyl benzene sulfonate detergent having 10 to 20 carbon atoms in its alkyl group in the hot mixture and cooling the solution to form a macroscopically homogeneous solid, the proportions of the components in the solution being 40 to 60 parts by weight of wax, 1 to 10 parts by weight of a fatty acid containing 10 to 20 carbon atoms per molecule and 60 to 40 parts by weight of sulfonate.

## References Cited in the file of this patent

## UNITED STATES PATENTS

|           |           |                |
|-----------|-----------|----------------|
| 2,175,285 | Duncan    | Oct. 10, 1939  |
| 2,356,903 | Wood      | Aug. 29, 1944  |
| 2,462,758 | Malkemus  | Feb. 22, 1949  |
| 2,653,913 | Van Dijck | Sept. 29, 1953 |
| 2,678,921 | Turck     | May 18, 1954   |

## FOREIGN PATENTS

|         |               |                |
|---------|---------------|----------------|
| 583,028 | Great Britain | Dec. 5, 1946   |
| 592,206 | Great Britain | Sept. 10, 1947 |